

Nov. 22, 1932.

W. H. WAGGAMAN ET AL

1,888,896

PRODUCTION OF PHOSPHORUS AND PHOSPHORIC ACID

Filed March 21, 1930



Inventors

W. H. WAGGAMAN  
AND S. D. GOOCH

Denniss & Sonnes

Attorneys

## UNITED STATES PATENT OFFICE

WILLIAM H. WAGGAMAN, OF LAKELAND, AND STAPLETON D. GOOCH, OF LAKE WALES,  
FLORIDA, ASSIGNORS TO CORONET PHOSPHATE COMPANY, OF NEW YORK, N. Y., A  
CORPORATION OF NEW YORK

## PRODUCTION OF PHOSPHORUS AND PHOSPHORIC ACID

Application filed March 21, 1930. Serial No. 437,748.

This invention relates to the production of phosphorus and phosphoric acid and more particularly to an improved method of and apparatus for the pyrolytic reduction of phosphatic material.

A well-known and widely used method of preparing phosphorus and phosphoric acid from phosphatic material comprises charging a mixture of this material with a siliceous flux and a suitable fuel to a fuel furnace of the blast furnace type. At the high temperatures of operation the silica displaces the phosphoric acid of the rock to form phosphorus pentoxide or, if reducing conditions are maintained, elemental phosphorus.

While blast furnaces have heretofore been employed for this volatilization process, little attention appears to have been paid to the general problem of modification of the construction and design so as to secure more efficient results. Blast furnaces of standard size and construction have been employed which conform generally to that type used in the manufacture of pig iron and ferro alloys. Little has been done to modify such constructions in light of the problems peculiar to the production of phosphorus by this method. In the usual type of apparatus the ratio of the height (from the hearth to the stock line) to the diameter of the furnace crucible has not been over seven to one; as a matter of fact, this ratio rarely exceeds six to one. This limitation in the height of the furnace seems to be due to the prevalent belief that an increase in this ratio is impractical because of the disadvantages resulting from the increased weight of stock and increase in resistance to the passage of gases. We have found that by specially designing a blast

furnace and thereby departing from the conventional structures, and furthermore by subjecting the material to be treated in the furnace to a special preliminary treatment, new and improved results can be secured.

It is a major object of the present inven-

tion, therefore, to provide an improved blast furnace so designed as to effectively and economically produce phosphorus and/or phosphoric acid.

Another object is to provide an improved process for producing phosphorus by the pyrolytic method by which high fuel economies are achieved.

A further object is to provide a process for producing phosphorus, of a relatively high degree of purity, by the pyrolytic method.

With these and other equally important objects in view, the invention comprehends the special preliminary treatment of a charge of phosphatic material and the smelting of this charge in a blast furnace so constructed and designed as to present a relatively high column of stock.

In order to more clearly explain the invention, there is shown in the accompanying drawing, an illustrative embodiment of the apparatus employed.

This may comprise a blast furnace of any desired construction but having a certain predetermined ratio of height to width and/or area of stock space, as explained more fully hereinafter.

As shown in the drawing, such a furnace may in its general features of construction, conform to the usual type having a tapered shaft and belly of large diameter. More specifically, it may comprise, as shown, a mantle or outer stack casing which is of any desired material, provided with a shirt or lining 2 of some refractory such as fire brick. If desired, a stuffing of sand or other suitable material or a second lining, may be interposed between the mantle and shirt.

The casing structure may be sustained by any suitable type of supporting means, as indicated conventionally on the drawing by the supporting elements 3. The complete casing encloses the shaft or fire room 4, which may taper, upon any predetermined inclination from the mouth to the belly. Below the belly,

the shaft may be constricted in accordance with any approved design to present the boshes 5, the subjacent hearth and crucible sections 6 and 7, respectively. The crucible 5 may be apertured adjacent the base or sole 8 to provide a tap hole 9, through which the fused slag may be withdrawn.

Connected with any suitable source of hot air, is a conduit 10, which feeds the tuyères 11. These, in the well-known manner, feed highly preheated air to the mass to be smelted so as to effect the combustion of the carbonaceous fuel.

Positioned in the upper section of the furnace is a means for feeding the charge thereto. For the purpose of simplifying the drawing, this is shown as a conventional bell and hopper 12, the end of which terminates over a feed hole 13, which latter communicates, as 20 shown, with the shaft. It will be understood that the element 12 is given as indicative of any suitable type of feeding mechanism. It will also be appreciated that the feeding shaft 13 may be provided with any suitable type of 25 check mechanism, so as to prevent escape of gases through the feeding conduit. Also positioned in the upper section of the furnace is the gas draw-off or downcomer 14, through which the gaseous products of combustion are 30 withdrawn. These gases may be subjected to any desired type of subsequent treatment such, for example, as is described in co-pending application, Serial No. 434,142 filed Mar. 7, 1930.

35 We have found, as indicated hereinbefore, that improved results may be secured if the ratio of the height of the stack, as measured from the hearth to the furnace stock line to the diameter of the furnace crucible, is increased so as to present a relatively high 40 column of stock. This is particularly true if the phosphatic material is subjected to a preliminary treatment. In the preferred operation the phosphatic raw material is first 45 sintered so as to provide a relatively light interstitial mass of phosphate and siliceous material.

We have found further that if the above 50 mentioned ratio, i. e., the height from the hearth 6 to the furnace stock line 15, bear a relationship of between seven and eight and one-half to one the width of the crucible 7, improved results are secured.

This additional height of stock column is 55 very desirable. In the first place by providing a higher stack, the time element for the absorption of heat by the phosphatic material by the furnace gases is increased, and the furnace gases are withdrawn and the phosphatic charge enters the reaction zone of the furnace at a temperature at which phosphorus is almost immediately evolved. In addition, the porous and permeable nature of an expanded or sintered charge presents much 60 less resistance to the passage of gases than

does a heavier and more compact charge, and particularly where the latter is quite dense, as in the case of briquettes and lumps of natural phosphate rock. When using a porous charge of relatively greater height, the increase in gas velocity due to the porosity of the charge is offset by providing a higher column of stock, a longer path for the furnace gases, and an increase in the heat exchange area.

Furthermore, on account of the high temperatures employed in smelting phosphate rock and siliceous material, a considerable amount of fumes and volatile products are evolved. By providing a longer column of stock through which the furnace gases can percolate or filter, a greater amount of these evolved materials are filtered out; that is to say, the longer stock column acts as a condensing or filtering medium to retain finely divided products and impurities which, if passing off with the phosphorus, would adversely affect the value of the product.

It will be appreciated, furthermore, that by mixing carbonaceous fuel with the light 50 sintered charge, a wider dispersion of a given quantity of fuel per volume of phosphatic material is secured. As the result of this, the combustion of the fuel is accelerated and rendered more complete. In other words, 55 optimum utilization is made of fuel values and the heat generated by the combustion of the fuel is more evenly and uniformly disseminated through the mass to be smelted.

In the preferred construction, therefore, we employ a furnace of a blast furnace type of such dimension that the ratio of its height (from the base of the crucible to the stock line) to the inside diameter of the crucible is at least seven and one-half to one. A typical example of such a structure is shown in the drawing in which a furnace having a distance of ninety feet from the crucible to the stock line, has a crucible or hearth diameter of twelve feet instead of seventeen feet, as is the usual width in a furnace of such a height.

In carrying out the process, a sintered mass of phosphate and siliceous material, is mixed with a predetermined quantity of coke or other carbonaceous material and is fed to the blast furnace through the bell and hopper 12, or equivalent feeding means. If desired, of course, the sintered phosphatic material and the fuel may be fed into the top of the furnace through separate elements and at respectively correlated and predetermined rates. During operation, a blast of air preheated to at least 1400° F. is fed through the tuyères in the well-known manner. The gaseous mixture and phosphorus vapor evolved by this treatment passes upwardly through the long column of stock and is discharged through downcomer 14, and thence through a dust catcher of conventional design. The phosphorus and any solid parti-

cles still contained in the gases are then condensed out and treated to prepare phosphoric acid as, for example, in the manner described in the copending application above referred to.

5 It will now be appreciated that we have provided an improved process and apparatus for preparing phosphorus by the pyrolytic method. By accurately correlating the physical character of the charge with respect to 10 the area within the zone of action, improved results are secured. The expanded or interstitial nature of the charge is fully utilized to subserve the function of largely separating out or filtering solid particles, thereby diminishing the load on the purifying apparatus. The height of the charge is so regulated that optimum absorption of the sensible heat of 15 the furnace gases is secured. This factor is of peculiar importance in the production of phosphorus because of the high temperature of 20 operation.

The thermal units required to smelt, a charge of phosphatic material and to reduce 25 and volatilize the phosphorus are much greater than those required in other blast furnace operations such, for example, as the production of pig iron and ferro alloys. It will be appreciated, in the present process, that these 30 thermal economies are attributable in part to the physical character of the stock and in part to its dimensional characteristics: thus the permeable nature of the charge permits a relatively free passage of the gases and thus 35 insures more uniform heating in the upper portions of the column; the porosity of the charge assures a high rate of area to volume and hence increases the heat contacting or transfer surface; the elongated or extenuated 40 character of the stock (with respect to the direction of flow of the gases) provide an increased or protracted time of contact between the hot gases and the charge, and thereby appreciably increases the total heat absorption.

45 In short, these improved advantages are achieved by the correlation of the physical character of the charge and the dimensional characteristics of the charge as determined 50 and fixed by the improved design of the furnace.

55 It is to be understood, therefore, that while the typical apparatus has been shown in the drawing and described in the specification, it is to be understood that this is given merely for purposes of illustration and is to be considered as typical of any similar furnace structure which, in conjunction with the described physical character of the charge, will 60 insure the described beneficial results.

We claim:

65 A method of pyrolytically producing phosphorus from phosphatic material comprising charging a mixture consisting of a sintered mass of phosphate and siliceous material to-

gether with a fuel into a furnace zone, building the charge in the furnace zone until the height of the charge bears a ratio to the width of the charge of more than seven and one-half to one, igniting the charge and passing 70 the generated gases and vapors upwardly through the elongated column-like charge, the height of which is more than seven and one-half times the width, thereby effecting a high flow velocity of the gases and vapors 75 and insuring a prolonged heat exchange period between the hot evolved gases and vapors and the upper section of the charge.

In testimony whereof we affix our signatures.

WILLIAM H. WAGGAMAN.  
STAPLETON D. GOOCH.

80

85

90

95

100

105

110

115

120

125

130